

Patented Nov. 16, 1926.

1,607,482

# UNITED STATES PATENT OFFICE.

MICHEL RUDIE, OF NEW YORK, N. Y.

## SURFACE ORNAMENTATION.

No Drawing.

Application filed May 4, 1925. Serial No. 27,890.

This invention relates to the ornamentation of paper, cardboard, wood or other surfaces.

The objects of the invention are to ornament such surfaces without impairing the same, to secure beautiful and striking color effects at a reasonable cost, without using varnish, expensive oils, gums, injurious acids or the like, and without requiring special equipment or complicated treatment.

These objects are attained by certain novel methods of treatment and combinations of elements as hereinafter set forth and broadly claimed.

One of the special features of the invention is the bringing together on the surface to be ornamented, different colors of chemically repellent nature and causing them to react in such a way as to establish on the surface, variegated boundaries or patterns simulating tapestry art work. As a practical example, I have taken the aniline colors, brown and red, which are chemically repulsive, in the sense that they are immiscible or only partly miscible, and have applied these colors by a brush or the like in contiguous relation on a surface of paper or cardboard. As these colors contact along the lines of contiguity, a repulsive reaction takes place in which the deeper constituents of the two colors are thrown outward and meeting, form a jagged border, outlining in a general way, the shape of the color areas. These areas may be of irregular outline in the nature of splotches or they may be of regular outline, such as to form stripes or bars, but in each instance, the repulsive action serves to set up a darker border outlining the areas and giving a heightened color effect. The repulsive action takes place only where the colors come in contact and only while they are in the wet state and hence while their chemically repellent characteristics are most active.

By using different varieties of colors having these inherently repulsive characteristics, innumerable color combinations can be produced in regular or irregular designs and with the color areas of large or small size, the color figures in each instance being outlined with a distinctive border giving the tapestry effect.

A metallic effect can be produced by combining certain of the antagonistic colors which in their reaction create "high lights" having a bronze or gold effect. As practical

examples, I combine malachite green with basic green or blue, acid green with malachite green, basic violet with any of the direct colors. Thus the brilliancy of metallic effects are produced without using any metallic powders or liquids.

To brighten the effect, a crystallized surface may be provided by applying over the colors or using with them, a coating solution made up for instance of copper, zinc and stannous sulphates combined with magnesium sulphate in a solution of dextrine or casein, sugar and glycerine. This quickly dries as a crystalline coating at room temperature, no special heat treatment being required, and it being unnecessary to use any acids or alkalis.

The crystallization may be prevented at any point or points on the surface by rendering the color used at such point or points chemically adverse to crystallization as by combining with it, a small proportion of sulphuric, nitric or acetic acid. In such instance these chemically adverse spots remain free of crystals while the rest of the surface is covered with the crystalline coating. In this way it is possible to use the crystals as a background, outlining other non-crystalline portions.

The crystallized surface forms a glossy light reflecting coating sufficiently permanent under ordinary conditions but it does not injure the paper or other surface and may be washed off with water or other solvent, leaving the paper smooth and uninjured.

I have found in my numerous experiments that the acid, basic and direct dyes, and some of the chrome dyes are antagonistic one to another, that is, the acid colors are repugnant to the basic colors, the basic colors are repugnant to the direct colors and even some of the chrome colors are repugnant to each other, in the manner above described, such as by their repellent action to create the irregular boundary lines producing the tapestry effects.

For the crystallized surface, I have used a solution of several metallic sulphates such as nickel, zinc, tin, aluminum, cupric, combined in dextrine or glue, sugar and glycerine, with an added quantity of magnesium sulphate or lead acetate. The magnesium sulphate or lead acetate, however, is not essential. The crystallization takes place naturally at practically any temperature and

the crystallized surface is not affected by temperatures to which the coated surfaces would ordinarily be subjected. Various colors may be combined with these sulphates.

5 In many cases a double salt solution is used, for example, nickel sulphate and zinc sulphate, nickel and magnesium sulphates or cupric and magnesium sulphates. Where in such a case one of the sulphates is of a 10 more or less fugitive character, such as zinc and magnesium sulphates, the combination with the other sulphate appears to overcome that fugitive character and forms a more lasting crystalline surface 15 which is non-oxidizing and so not affected by air, retains its iridescent appearance and is not injured by dampness or handling with moist fingers.

The crystallizing compound may be made 20 up as a solution and applied to the paper or other surface whenever required. The paper ornamented with the tapestry effect or with the crystallized surface, or combinations of both, is adapted for many purposes, such as for covering boxes and the like 25 and the fact that such ornamentation is applicable directly to cardboard makes it possible to ornament cardboard boxes and the like by applying the ornamentation to the 30 cardboard, instead of to a separate paper cover, as has been the practice heretofore.

By combining several colors in the crystallizing solution, the effects of polarized light 35 can be produced, said colors appearing on the surface to which they are applied as a crystalline light reflecting coating having a "changeable" color effect when viewed at different angles or under different lights.

What is claimed is:

40 1. The process of ornamenting the surface of paper or other material which comprises applying to such surface, dyes of chemically repellent nature in contiguous relation and thereby enabling said dyes in their antagonistic reaction to build up a border of heightened color outlining the division between the color areas.

45 2. The process of ornamenting the surface of paper or other material which comprises

applying to such surface, dyes of chemically 50 repellent nature in contiguous relation and thereby enabling said dyes in their antagonistic reaction to build up a border of heightened color outlining the division between the color areas and applying to said 55 color areas, a self-crystallizing compound of metallic sulphates.

3. The process of ornamenting the surface of paper or other material which comprises applying to such surface, dyes of chemically 60 repellent nature in contiguous relation and thereby enabling said dyes in their antagonistic reaction to build up a border of heightened color outlining the division between the color areas and applying to said 65 color areas, a self-crystallizing compound of metallic sulphates and preventing the crystallization at certain portions of the surface by previously rendering such portions chemically adverse to crystallization. 70

4. The process of producing metallic effects in surface ornamentation without the use of metallic materials which comprises applying to the surface to be ornamented, a combination of dyes having chemically repellent characteristics. 75

5. As a new article of manufacture, paper having applied to the surface of the same, a crystallized coating of metallic sulphates combined with a dye. 80

6. As a new article of manufacture, paper material having applied directly to the surface of the same, a crystalline coating of at least two different metallic sulphates combined with a dye, said coating being of a 85 lasting flexible nature and providing in its colored crystalline composition, an iridescent changeable color effect when exposed to the light.

7. The process of producing iridescent 90 color effects on paper comprising applying to the surface of the paper, a crystallizable double sulphate solution of metallic salts containing a dye and permitting said colored salt solution to crystallize on the paper. 95

In witness whereof, I have hereunto set my hand this 2nd day of May, 1925.

MICHEL RUDIÉ.